# EUROPEAN PATENT SPECIFICATION

(11) **EP 1 230 325 B1**
(45) Date of publication and mention of the grant of the patent: **11.01.2006**
(21) Application number: 00971389.2
(22) Date of filing: 17.10.2000
(51) Int. Cl.: C10L 1/04, C10L 1/08

(54) **FUEL OIL COMPOSITIONS WITH IMPROVED COLD FLOW PROPERTIES**
BRENNSTOFFÖLZUSAMMENSETZUNG MIT VERBESSERTEN KALTFLIESSEIGENSCHAFTEN
COMPOSITIONS DE PRODUIT PETROLIER PRESENTANT DES PROPRIETES DE FLUAGE A FROID AMELIOREES

(30) Priority: 29.10.1999 GB 9925643
(43) Date of publication of application: 14.08.2002
(73) Proprietor: ExxonMobil Research and Engineering Company, Annandale, NJ 08801 (US)
(72) Inventor: COCHRANE, Heather, D., New Jersey 08003 (US); CLOKE-BROWNE, Veronica, Hants SO21 1PT (GB)
(74) Representative: Troch, Geneviève
(86) International application number: PCT/EP2000/010185
(87) International publication number: WO 2001/032810

(56) References cited:
- US-A- 2 717 858
- US-A- 2 892 769

## Description

This invention relates to fuel oil compositions, especially middle distillate fuel oil compositions, with improved flow properties.

It is important that fuel oil compositions, especially middle distillate oil compositions such as automotive diesel oils, heating oils and gas oils (hereafter collectively referred to as "fuel oil" for convenience) retain their flow properties at relatively low temperatures. The main cause of such loss of flow properties is due to the formation of wax which tends to precipitate out and agglomerate thereby plugging burner and vehicle fuel filters and hence impairing flow. The temperature at which the wax starts to appear is termed the cloud point of the fuel. The cold filter plugging point (CFPP) is recognised as a measure of the operability of a fuel and the temperature at which a fuel will start to block vehicle filters. It is generally less than or equal to the cloud point of the fuel. This problem has been well recognized in the art and has hitherto been mitigated by the use of various flow improving additives also known as middle distillate flow improvers (MDFI) which reduce the CFPP of responsive fuels. One such example is Paraflow® 240 (commercially sold by Infineum). The flow improvers can change the size or the shape of the crystals as they precipitate out of the oil at low temperatures thereby allowing them to pass through the vehicle filter easily and avoid blockage of the fuel filter of the vehicle. Either way, it is important that the flow properties of the fuel oils are maintained.

Hitherto, crude oil was refined into motor gasoline, automotive diesel oils (hereafter "ADO") and gas oils used as heating oils (fuel oils) and their respective specifications were such that it was possible to easily treat ADO, gasoil and heating oils. However, recent legislation to minimise the amount of sulphur and also constrain other properties, eg density, in ADOs has meant that some of the heavier components of ADOs, such as e.g. catalytically cracked heating oils, have been displaced into the gasoil and heating oil fractions. These changes in the composition of ADO, gasoils and heating oils may mean that the effectiveness of conventional cold flow improvers such as Paraflow® 240 is lessened.

It is an object of the present invention to improve the flow properties of fuel oils (as herein defined) containing conventional flow improvers by incorporating therein a heavy catalytically-cracked naphtha.

Accordingly, the present invention is a fuel oil composition according to claim 1.

In the fuel compositions of the present invention, the various components referred to are all derivable from various process streams of a petroleum crude refinery process. Such methods are well known in the art and are described in detail, for instance, by Keith Owen and Trevor Colley in "Automotive Fuels Reference Book", Second Edition, published by the Society of Automotive Engineers, Inc, Warrendale, PA, USA (1995). Specifically referred to are Chapter 3 of this text-book at pages 29-49 and Chapter 16 at pages 419-469 and 865-890, the latter pages forming Appendix 12 which is a 'Glossary of Terms' used in this art.

Fraction (c) suitably has an aromatics content in the range from about 60 - 75% by weight.

The fuel oil compositions of the present invention may contain in addition other conventional distillate fractions from a petroleum crude refinery process under atmospheric or vacuum conditions. These include *inter alia* components (d) to (g) described below:
(d) A fraction from a vacuum pipestill which suitably has a boiling point in the range from about 200 to 400°C, preferably from about 240-365°C. This fraction (d) is suitably present in the compositions of the present invention in an amount ranging from about 3-7% by weight, preferably from about 4-6 % by weight of the total composition.
(e) A fraction from an atmospheric pipestill which suitably has a boiling point in the range from about 160-380°C, preferably from about 183 to331°C. This fraction (e) is suitably present in the compositions of the present invention in an amount ranging from about 5 to 15% by weight, preferably from about 9 to 10% by weight, typically about 9.5-10.0% by weight.
(f) A fraction from an atmospheric pipestill which suitably has a boiling point in the range from about 230 -350°C, preferably from about 231 to 344°C. This fraction (f) is suitably present in the compositions of the present invention in an amount ranging from about 15 to 30% by weight, preferably from about 20-25% by weight.
(g) A fraction from an atmospheric pipestill which suitably has a boiling point in the range from about 210-420°C, preferably from about 216 to 395°C. This fraction is suitably present in the compositions of the present invention in an amount ranging from about 3 to 8% by weight, preferably from about 4-6 % by weight.

The fuel oil compositions of the present invention having an n-paraffin (C₁₂₊) content of less than 20% by weight particularly benefit by blending with the light naphtha fraction (c). Such fuel oil compositions suitably have a cloud point of about -3 to-4°C.

The cold flow additive in fuel oil composition is suitably one that is generally available provided it is soluble in the fuel oil composition, although copolymers of ethylene and at least one other unsaturated monomer which may be an additional monoolefin or an unsaturated ester such as eg vinyl acetate, vinyl propionate, vinyl butyrate, ethyl acrylate and lauryl methacrylate or the like. The other unsaturated monomer can also be a mixture of an unsaturated mono-ester or diester and a straight chain or branched chain α-monoolefin. Mixtures of copolymers, such as eg a copolymer of ethylene and vinyl acetate with an alkylated polystyrene or with an acylated polystyrene, can also be used. Where the flow additive is a coolymer, it suitably consists of 1 to 40, preferably 1 to 20 and more preferably 3 to 20 molar proportions of ethylene per molar proportion of the other unsaturated monomer. The additive copolymer is suitably oil-soluble and has a number average molecular weight in the range from about 1,000 to 50,000, preferably about 1,000 to about 5,000. The cold flow additive is preferably an ethylene-vinyl carboxylate copolymer which may be selected from one or more of Paraflow®240, Paraflow® 226, Paraflow® 222, Paraflow® 275, Paraflow® 255, Paraflow® 223, Paraflow® 332, Paraflow® 209, Paraflow® 206, Paraflow® 480, Paraflow® 482, Paraflow® 479 (all ex Infineum), KF 6100S, KF 6100, KF 6301, KF 6101 (ex BASF), and DF 4842 (ex Clariant). Some of these oil-soluble additives which are eg olefin/vinyl carboxylate copolymers having a number average molecular weight as measured by vapour pressure osmometry of 1,000 to 10,000 which may optionally contain polar nitrogen compounds as co-additives, are described in EP-A-261957 and WO 94/00535.

The surprising feature of the present invention is that component (c), which is a relatively light fraction compared to the distribution of heavier components in fuel oils, is able to improve the effectiveness of conventional cold flow improvers in such fuel oils. It has been found that by using an aliquot of component (c) in the fuel oil compositions, it is possible to depress the cloud point and the temperature of operability, the latter as determined by the cold-filter plugging point (hereafter "CFPP") to a significant extent.

The present invention is further illustrated with reference to the following Examples:

### EXAMPLES:

The following data was generated by subjecting a variety of fuel oils, each of which contained (i) 500 ppm by volume of an ethylene-vinyl acetate copolymer (Paraflow® 240, ex Infineum) cold flow additive and (ii) a 1050 ppm by volume of a gasoil marker dye, to a cold flow plugging point (CFPP) test. The test is described in detail in the text-book by Owen & Coley referred to above at pages 422-426 in Chapter 16.1.5. This is an IP 309 test and is also published as a European Standard by CEN, EN 116:1981. Briefly, 40 ml of a sample of the test oil is cooled by a bath maintained at about -34°C. Periodically (at each 1°C drop in temperature starting from not less than 5°C above the cloud point thereof), the cooled oil is tested for its ability to flow through a fine screen in a given time period. This cold flow property is tested with a device consisting of a pipette the lower end of which is attached an inverted funnel positioned below the surface of the test oil. Stretched across the mouth of the funnel is a 350 mesh screen having an area of about 2.90 cm² (0.45 in²). The periodic tests are each initiated by applying a vacuum to the upper end of the pipette whereby oil is drawn through the screen up into the pipette to a mark indicating 20 ml. The test is repeated with each I °C drop in temperature until the oil fails to fill the pipette up to that 20 ml mark within 60 seconds. The temperature at which the last filtration commenced is recorded as the CFPP.

**TABLE**

| Components | Fuel Composition 1* (Wt %) | Fuel Composition 2 (Wt %) | Fuel Composition 3 (Wt %) |
|---|---|---|---|
| Component (g) | 4.9 | 4.9 | 4.9 |
| Component (e) | 9.9 | 9.9 | 9.9 |
| Component (a) | 16.2 | 8.4 | 5.0 |
| Component (c) | - | 7.8 | 15.0 |
| Component (b) | 42.2 | 42.2 | 38.4 |
| Component (f) | 21.8 | 21.8 | 21.8 |
| Component (d) | 5.0 | 5.0 | 5.0 |
| **Total** | 100 | 100 | 100 |
| Cloud point (°C) | -3 | -4 | -4 |
| CFPP (°C) | -8 | -10 | -15 |

The above results show that partially replacing some of the conventional gas oil components in fuel oils with light naphtha fraction from the catalytic cracking of heavy gasoil clearly improves the CFPP of the fuel oils to a significant extent.

## Claims

1. A fuel oil composition derived from petroleum crude refinery process comprising:
(a) 5-18 % by weight of the total fuel composition of a heavy fraction produced by catalytic cracking of heavy gas oil from the atmospheric or vacuum pipestill, having a boiling range from 184 to 376 °C,
(b) 35-45 % by weight of the total fuel composition of a gasoil product from an atmospheric pipestill, having a boiling range of from 244 to 330°C,
(c) 5-15 % by weight of the total composition of a light naphtha fraction obtained by catalytic cracking of heavy gasoil from atmospheric or vacuum pipestill, having a boiling point in the range from 136 to 231°C,
said fuel oil composition further comprising from 0.001 to 2 % by weight of the total fuel oil composition of a cold flow additive,

2. The composition according to claim 1, wherein the light naphtha fraction has aromatics content in the range of from 60 to 75 % by weight.

3. The composition according to claim 1 or 2, containing in addition one or more distillate fractions selected from:
(d) a fraction from a vacuum pipestill having a boiling point in the range from 200 to 400°C and being present in an amount ranging from 3 to 7% by weight;
(e) a fraction from an atmospheric pipestill having a boiling point in the range from 160 to 380°C and being present in an amount ranging from 5 to 15% by weight;
(f) a fraction from an atmospheric pipestill having a boiling point in the range from 230 to 350°C and being present in an amount ranging from 15 to 30% by weight; and
(g) a fraction from an atmospheric pipestill having a boiling point in the range from 210 to 420°C and being present in an amount ranging from 3 to 8% by weight.

4. The composition according to any one of claims 1 to 3, wherein
• fraction (d) has a boiling point in the range from 240 to 365°C;
• fraction (e) has a boiling point in the range from 183 to 331°C;
• fraction (f) has a boiling point in the range from 231 to 344°C; and
• fraction (g) has a boiling point in the range from 216 to 395°C.

5. The composition according to any one of claims 1 to 4, wherein the cold flow additive is an ethylene vinyl acetate copolymer

6. A method of improving the cold flow properties of a fuel oil composition derived from petroleum crude refinery process comprising from 0.001 to 2.0 % by weight of the total fuel oil composition of a cold flow additive and the following components from the refinery process:
a) a relatively heavy fraction from a catalytically cracked heavy gasoil in turn derived from an atmospheric or vacuum pipestill, said fraction having a boiling range of 180 to 380°C and being present in an amount of 3 to 20% by weight, and
b) a gasoil product from an atmospheric pipestill, said product having a boiling range of 240 to 335°C and being present in an amount of 30-50% by weight,
said method comprising replacing at least partially components (a) and/or (b) in said composition by at least one relatively light naphtha fraction (c) from an atmospheric or a vacuum pipestill, said light fraction (c) having a boiling range of 130 to 235 °C and being present in the improved fuel oil composition in an amount of 3 to 20% by weight, in such a way that fractions (a) and (b) are present in the improved fuel oil composition respectively in an amount ranging from 5 to 18 % by weight and from 35 to 45 % by weight, all weights being based on the total weight of the fuel oil composition.

## Patentansprüche

1. Brennstoffölzusammensetzung, die aus einem Rohölraffinerieverfahren abgeleitet ist, umfassend:
(a) 5-18 Gew.-% der Gesamtbrennstoffzusammensetzung von einer schweren Fraktion, die durch katalytisches Cracken von schwerem Gasöl aus dem atmosphärischen oder Vakuumröhrenofen produziert worden ist, mit einem Siedebereich von 184 bis 376°C,
(b) 35-45 Gew.-% der Gesamtbrennstoffzusammensetzung von einem Gasölprodukt aus einem atmosphärischen Röhrenofen mit einem Siedebereich von 244 bis 330°C,
(c) 5-15 Gew.-% der Gesamtzusammensetzung von einer leichten Naphthafraktion, die durch katalytisches Cracken von schwerem Gasöl aus atmosphärischem oder Vakuumröhrenofen produziert worden ist, mit einem Siedebereich von 136 bis 231°C,
wobei die Brennstoffölzusammensetzung ferner 0,001 bis 2 Gew.-% der Gesamtbrennstoffölzusammensetzung von einem Kaltfließadditiv umfasst.

2. Zusammensetzung nach Anspruch 1, bei der die leichte Naphthafraktion einen Aromatengehalt im Bereich von 60 bis 75 Gew.-% hat.

3. Zusammensetzung nach Anspruch 1 oder 2, die zusätzlich eine oder mehrere Destillatfraktionen enthält, die ausgewählt sind aus:
(d) einer Fraktion aus einem Vakuumröhrenofen mit einem Siedepunkt im Bereich von 200 bis 400°C, die in einer Menge im Bereich von 3 bis 7 Gew.-% vorhanden ist;
(e) einer Fraktion aus einem atmosphärischen Röhrenofen mit einem Siedepunkt im Bereich von 160 bis 380°C, die in einer Menge im Bereich von 5 bis 15 Gew.-% vorhanden ist;
(f) einer Fraktion aus einem atmosphärischen Röhrenofen mit einem Siedepunkt im Bereich von 230 bis 350°C, die in einer Menge im Bereich von 15 bis 30 Gew.-% vorhanden ist;
(g) einer Fraktion aus einem atmosphärischen Röhrenofen mit einem Siedepunkt im Bereich von 210 bis 420°C, die in einer Menge im Bereich von 3 bis 8 Gew.-% vorhanden ist.

4. Zusammensetzung nach einem der Ansprüche 1 bis 3, bei der
• Fraktion (d) einen Siedepunkt im Bereich von 240 bis 365°C hat;
• Fraktion (e) einen Siedepunkt im Bereich von 183 bis 331°C hat;
• Fraktion (f) einen Siedepunkt im Bereich von 231 bis 344°C hat;
• Fraktion (g) einen Siedepunkt im Bereich von 216 bis 395°C hat.

5. Zusammensetzung nach einem der Ansprüche 1 bis 4, bei der das Kaltfließadditiv Ethylen/Vinylacetat-Copolymer ist.

6. Verfahren zur Verbesserung der Kaltfließeigenschaften einer Brennstoffölzusammensetzung, die von einem Rohölraffinerieverfahren abgeleitet ist und 0,001 bis 2,0 Gew.-% der Gesamtbrennstoffölzusammensetzung von einem Kaltfließadditiv und die folgenden Komponenten aus dem Raffinerieverfahren umfasst:
a) eine relativ schwere Fraktion aus einem katalytisch gecrackten schweren Gasöl, das wiederum von einem atmosphärischen oder Vakuumröhrenofen abgeleitet ist, wobei die Fraktion einen Siedebereich von 180 bis 380°C hat und in einer Menge von 3 bis 20 Gew.-% vorhanden ist, und
b) ein Gasölprodukt aus einem atmosphärischen Röhrenofen, wobei das Produkt einen Siedebereich von 240 bis 335°C aufweist und in einer Menge von 30 bis 50 Gew.-% vorhanden ist,
wobei in dem Verfahren Komponenten (a) und/oder (b) in der Zusammensetzung mindestens teilweise durch mindestens eine relativ leichte Naphthafraktion (c) aus einem atmosphärischen oder einem Vakuumröhrenofen ersetzt werden,
wobei die leichte Fraktion (c) einen Siedebereich von 130 bis 235°C hat und in der verbesserten Brennstoffölzusammensetzung in einer Menge von 3 bis 20 Gew.-% vorhanden ist, so dass Fraktionen (a) und (b) in der verbesserten Brennstoffölzusammensetzung in einer Menge im Bereich von 5 bis 18 Gew.-% beziehungsweise 35 bis 45 Gew.-% vorhanden sind, wobei sich alle Gewichte auf das Gesamtgewicht der Brennstoffölzusammensetzung beziehen.

## Revendications

1. Composition d'huile combustible dérivée d'un procédé de raffinage de pétrole brut comprenant :
(a) 5 à 18% en poids de la composition totale de combustible d'une fraction lourde obtenue par craquage catalytique de gasoil lourd produit en four tubulaire atmosphérique ou sous vide, ayant une plage d'ébullition de 184 à 376°C,
(b) 35 à 45% en poids de la composition totale de combustible d'un gasoil produit en four tubulaire atmosphérique, ayant une plage d'ébullition de 244 à 330°C, et
(c) 5 à 15% en poids de la composition totale de combustible d'une fraction légère de naphta obtenue par craquage catalytique de gasoil lourd produit en four tubulaire atmosphérique ou sous vide, ayant un point d'ébullition dans la plage de 136 à 231°C, ladite composition d'huile combustible comprenant en outre 0,001 à 2% en poids de la composition totale d'huile combustible d'un additif de fluage à froid.

2. Composition selon la revendication 1, dans laquelle la fraction légère de naphta a une teneur en aromatiques dans la plage de 60 à 75% en poids.

3. Composition selon la revendication 1 ou 2, contenant en plus une ou plusieurs fractions de distillat choisies parmi :
(d) une fraction produite en four tubulaire sous vide ayant un point d'ébullition dans la plage de 200 à 400°C et présente en quantité dans la plage de 3 à 7% en poids;
(e) une fraction produite en four tubulaire atmosphérique ayant un point d'ébullition dans la plage de 160 à 380°C et présente en quantité de 5 à 15% en poids;
(f) une fraction produite en four tubulaire atmosphérique ayant un point d'ébullition dans la plage de 230 à 350°C et présente en quantité de 15 à 30% en poids; et
(g) une fraction produite en four tubulaire atmosphérique ayant un point d'ébullition dans la plage de 210 à 420°C et présente en quantité de 3 à 8% en poids.

4. Composition selon l'une quelconque des revendications 1 à 3, dans laquelle :
• la fraction (d) a un point d'ébullition dans la plage de 240 à 365°C;
• la fraction (e) a un point d'ébullition dans la plage de 183 à 331°C;
• la fraction (f) a un point d'ébullition dans la plage de 231 à 344°C; et
• la fraction (g) a un point d'ébullition dans la plage de 216 à 395°C.

5. Composition selon l'une quelconque des revendications 1 à 4, dans laquelle l'additif de fluage à froid est un copolymère d'éthylène et d'acétate de vinyle.

6. Procédé d'amélioration des propriétés de fluage à froid d'une composition d'huile combustible dérivée d'un procédé de raffinage de pétrole brut comprenant 0,001 à 2,0% en poids de la composition totale d'huile combustible d'un additif de fluage à froid et les composants suivants du procédé de raffinage :
a) une fraction relativement lourde d'un gasoil lourd craqué catalytiquement dérivé à son tour d'un four tubulaire atmosphérique ou sous vide, ladite fraction ayant une plage d'ébullition de 180 à 380°C et étant présente en quantité de 3 à 20% en poids, et
b) un gasoil produit par un four tubulaire atmosphérique, ledit produit ayant une plage d'ébullition de 240 à 335°C et étant présent en quantité de 30 à 50% en poids,
ledit procédé comprenant le remplacement au moins partiel des composants (a) et/ou (b) de ladite composition par au moins une fraction de naphta relativement légère (c) d'un four tubulaire atmosphérique ou sous vide, ladite fraction légère (c) ayant une plage d'ébullition de 130 à 235°C et étant présente dans la composition d'huile combustible améliorée en quantité de 3 à 20% en poids, de manière que des fractions (a) et (b) soient présentes dans la composition d'huile combustible améliorée en quantités situées respectivement dans la plage de 5 à 18% en poids et dans la plage de 35 à 45% en poids, tous les poids étant basés sur le poids total de la composition d'huile combustible.
